

## UNITED STATES PATENT OFFICE

2,205,887

## COLORING TEXTILE MATERIALS

Jean G. Kern, Hamburg, N. Y., assignor to  
 National Aniline & Chemical Company, Inc.,  
 New York, N. Y., a corporation of New York

No Drawing. Application June 2, 1938,  
 Serial No. 211,390

14 Claims. (Cl. 8—134)

This invention relates to improvements in the process of coloring textile fibrous materials wherein the material is subjected to conditions favoring reduction of the coloring agent. It relates more particularly to improvements in the processing of textile fibrous material whereby the reduction of coloring agents on such materials is inhibited. (The term "coloring" as used herein and in the claims is meant to include dyeing and printing.)

An object of the invention is to provide inhibitors having improved action against the reduction of coloring agents for textile fibrous material under reducing conditions.

Another object of the invention is to provide inhibitors having improved action against the reduction of vat dyes by the reducing agents generally used in dyeing and printing with vat dyes.

Further objects are the prevention of haloing and scratching in discharge printing processes, the prevention of marking-off in kier boiling, and the provision of a highly effective resist agent for resist printing.

Other objects of the invention will in part be obvious and will in part appear hereinafter.

According to the usual methods of vat dyeing with anthraquinone, indigoid, thioindigoid and related vat dyes and various sulfur dyes, the dyes are rendered soluble by reducing them to the leuco or reduced form in an alkaline medium. This conversion to the soluble leuco form is necessary in vat dyeing. However, in many cases it is desired to partly prevent this reduction. Examples of this are resist printing and dyeing under vat dyes, preventing undesirable facing effects in discharge printing, and preventing marking-off in the kier-boiling of previously printed or dyed fabrics.

In resist printing, a so-called "resist" is printed on the fabric which subsequently is either padded or top-printed with the desired dye in reduced or unreduced form. The function of the resist is to prevent the dye from penetrating and becoming fixed on the fabric during the subsequent operations employed for fixing the dye. In general, compounds which prevent reduction of the dye are employed as the resists. While the process is more generally employed in connection with vat dyes, it is applicable also to sulfur colors, basic colors, and other dyestuffs which are frequently applied to fabrics in their reduced form.

In discharge printing of fabrics, a dischargeable (reducible) dye is first applied to the fabric and then certain discharge agents, usually reducing compounds incorporated into a discharge

paste, are printed on the fabric in the places where it is desired to destroy the color. In practicing this discharge printing, several difficulties are often encountered. If there is an excess of the discharge agent in the discharge paste, a flushing or creeping out into the fabric beyond the design takes place, forming borders or "halos" around the print (so-called "haloing"). If all of the discharge printing paste is not completely scraped off of the printing roller by the doctor blade, the color is discharged along other lines than the desired design. A similar difficulty is encountered when a solid particle gets under the doctor blade (so-called "scratching"), or when the printing paste is too thick, a thin film of discharge paste or "tarnish" being formed on the roller which is printed on the fabric and dulls or partially discharges and weakens the ground color (so-called "facing").

Fabrics containing multi-colored effect threads produced with vat or sulphur dyes or printed goods are sometimes kier-boiled after weaving or printing. In this process, contact between the white and colored-effect threads or between part of the goods which has been printed and other unprinted parts frequently causes a partial transfer of the dye from the colored to the other portion of the goods. This is called "marking off." A similar bleeding effect is often produced in mercerizing fabric containing vat or sulphur-dyed effect threads; also on mercerizing completely vat dyed fabrics a lightening of the color sometimes occurs. These effects are apparently caused by the vat or sulphur dye being slightly reduced under the alkaline conditions in the kier or mercerizer, so that it becomes partially dissolved.

It has been attempted to remedy these difficulties with moderate success by the use of such substances as nitroaromatic sulfonic and carboxylic acids in dilute alkaline solutions, as well as phenolic compounds capable of developing a quinoid structure in alkaline solution, for instance, para-nitrophenol. Thus, mononitro- and dinitro-benzene, toluene, phenol, and naphthol sulfonates have been heretofore proposed as inhibitors of the undesired reduction.

According to the present invention nitroaralkyl side-chain sulfonates are employed as reduction inhibitors in connection with the coloring of textile fibrous materials. As employed herein and in the claims the term "nitroaralkyl side-chain sulfonates" denotes aralkyl compounds containing at least one nitro group as a substituent in the aryl nucleus and at least one sul-

5 fonic acid group or salt thereof as a substituent in the alkyl group, the term "sulfonates" generically including the free sulfonic acids and their salts. I have found if the sulfonate group is attached to an open-chain aliphatic radical which in turn is attached to an aromatic radical containing a nitro group, and especially if the sulfonate group is attached to a nitrobenzyl radical, that the efficiency of the sulfonate as a reduction 10 inhibitor is far greater as compared to the sulfonates and carboxylates of nitroaromatic compounds in which the sulfonate or carboxylate group is a nuclear substituent.

15 Thus I have found, in accordance with the present invention, that extremely low percentages of sodium 4-nitro-benzyl sulfonate entirely prevent marking off in kier-boiling, efficiently resist the printing and fixation of vat dyes and other reducible dyes, and entirely nullify the 20 effect of excess undesired discharge agent.

25 A cross-dyeing effect is produced if the warp threads of any fabric are pretreated with a dilute solution of any of the nitro-aralkyl side-chain sulfonates of this invention and the fabric is subsequently printed with a vat dye in the regular manner. A unique effect of shading is thus obtained since the pretreated warp threads do not accept the vat dye while the filling presents the 30 vat dye coloring in its fullest development. The soluble nitro-aralkyl side-chain sulfonates may be applied to the warp threads during their sizing prior to weaving. Thus the nitro-aralkyl side-chain sulfonates may be dissolved in the sizing material or slashing liquor and applied to the 35 warp in the slasher in the regular manner.

35 The nitro-aralkyl side-chain sulfonates employed in accordance with the present invention may be represented by the following general formula:

40



45

where Ar is an aromatic radical, R is an aliphatic radical, preferably an aliphatic hydrocarbon radical, x and y are integers, and M is any cation. They include compounds in which the aromatic radical represented by Ar is free from further substituents or contains additional substituents; for instance, halogen and/or an alkyl, alkoxy, and/or a sulfo alkoxy group, etc. As examples 50 of such compounds, the following are mentioned:

2-nitro-4-chlor-1-phenoxyethyl sulfonic acid



55

4-nitro-1-methyl-2-phenoxyethyl sulfonic acid



60

4-nitro-2-methoxy-benzyl sulfonic acid



65

6-nitro-3-sulfo-ethoxy-benzyl sulfonic acid



70

nitro-phenyl-octyl sulfonic acid

nitro-phenyl-lauryl sulfonic acid

nitro-chlorphenyl-hexyl sulfonic acid

nitro-naphthyl-butyl sulfonic acid, etc.

I have found, however, that the most efficient compounds are those in which Ar is a benzene radical, R is a methylene group, x is 1 or 2, and y is 1. Thus, the following compounds have been found to yield superior results as reduction 5 inhibitors:

2-nitro-benzyl sulfonic acid

3-nitro-benzyl sulfonic acid

4-nitro-benzyl sulfonic acid

6-chlor-3-nitro-benzyl sulfonic acid

2,4-dinitro-benzyl sulfonic acid

4-chlor-3,5-dinitro-benzyl sulfonic acid

10

15

20

The nitro-aralkyl side-chain sulfonates may be employed in the form of the free sulfonic acids or in the form of the salts thereof; the particular form employed being selected with a view to the nature of the other reagents with which it is to be employed. In general the alkali-metal salts are employed in view of their superior solubility, and of these the sodium salts are preferably employed in view of their lower cost.

The amount of nitro-aralkyl side-chain sulfonate necessary to be employed for a given 25 purpose will vary with the conditions of the treatment of the material. The exact amount necessary in a given case can be easily determined by a trial dyeing or printing. Thus,  $\frac{1}{4}$  to 1 per cent aqueous solutions of the sodium salt 30 of 4-nitrobenzyl sulfonic acid generally are adequate for overcoming facing, haloing and scratching in discharge printing and in preventing marking off in kier-boiling and bleeding in mercerizing.

35

Several embodiments of the useful application of these compounds are discussed and shown in the following examples in which the parts are by weight. It is to be understood that these examples act merely as illustrations and not as 40 limitations of this invention.

#### Preventing mark-off in kier-boiling and mercerizing

Example 1.—1000 kilos of unbleached cotton 45 goods containing woven-effect threads dyed with vat dyes are boiled in a kier for 6 to 8 hours at 10 to 12 lbs. superatmospheric pressure in a solution composed of 3 per cent caustic soda (based on the weight of the goods), 1 per cent soda ash and  $\frac{1}{2}$  to 1 per cent of 4-nitro-benzyl sodium sulfonate. The goods are then soured, washed, bleached, soured, washed and dried in the usual way. No mark-off of the colored-effect threads 50 on the white threads is then obtained, because of the reduction inhibiting action of the nitrobenzyl compound.

55

60

Example 2.—Fabrics to be mercerized containing some vat dyed yarn are run on a mercerizing frame through a 25 per cent caustic soda 61 solution containing 1 to 2 per cent of 4-nitrobenzyl sodium sulfonate. The cloth should be travelling at a speed of about 60 yards per minute and be in the alkaline solution for about 30 seconds before the first wash. After-treatments 66 are performed in the usual way by souring with a 3 per cent sulfuric acid solution, rinsing and drying. It is found that there is no mark-off 7 effect or bleeding of the vat dyed yarn on the undyed threads. In the case of completely vat dyed fabrics no lightening of the color occurs.

#### Resist printing under vat dyes

A resist printing paste for obtaining a white 7 resist may contain from 150 to 180 parts of 4-

5 nitro-benzyl sodium sulfonate per 1000 parts of the usual paste. It is recommended, however, that from 60 to 80 parts of zinc acetate be added in order to convert the sodium salt into the less soluble zinc salt of the nitro-benzyl sulfonic acid thereby avoiding the running and flushing of the print color. The calcium salt also may be used in some instances to advantage.

10 *Example 3.*—Goods are printed with the following paste:

|                                 | Parts |
|---------------------------------|-------|
| Gum arabic                      | 300   |
| 4-nitro-benzyl sodium sulfonate | 175   |
| Kaolin                          | 55    |
| 15 Water                        | 390   |
| Zinc acetate                    | 80    |
|                                 | 1000  |

20 After printing, the goods are well dried, steamed for four minutes, then subsequently padded by passage through an alkaline hydrosulfite solution of a reduced vat dye, washed, soaped, rinsed and dried. The vat dye does not adhere to the 25 parts which have been printed, thus producing an excellent white resist on a vat dyed ground.

Amongst the vat dyes which may be resisted particularly well are to be mentioned:

|                                        | Color index |
|----------------------------------------|-------------|
| 30 Carbanthrene Yellow G               | 1118        |
| Carbanthrene Golden Orange 2RT         | 1097        |
| Carbanthrene Red BN                    | 1162        |
| Carbanthrene Olive G                   | 1150        |
| 35 Carbanthrene Blue BCS               | 1114        |
| Carbanthrene Blue 3G                   | 1109        |
| Brilliant Indigo 4B (Tetrabrom Indigo) |             |

40 *Example 4.*—Resists are obtained on warp yarns by running through a slasher box containing a mixture of potato starch and 5 per cent to 10 per cent of 4-nitro-benzyl sodium sulfonate. This sizing paste is then dried on the warps which are then woven into piece goods in the regular fashion. When these piece goods are printed or dyed with vat dyes, an excellent resist effect is obtained on the warp yarns.

#### Colored resists

50 The nitro-aralkyl sulfonate resist printing pastes may contain basic dyes or chrome dyes or azo components such as nitrosamines, diazo-amino compounds, etc. (for combination with coupling components on the fiber) whose dyeing 55 properties are unaffected by the presence of the nitro-aralkyl sulfonates in order to produce colored discharge effects.

55 Basic dyes are unaffected by nitro-aralkyl sulfonates and therefore may be effectively used to 60 produce colored resists under vat dyes. Basic dyes may be fixed by means of the conventional tannic acid and antimony salts or else in the form of their zinc lakes. In the first case, the cloth is printed with a printing paste containing 65 the nitro-aralkyl body, the basic dye, and tannic acid, the printed material subjected to steaming and then passed through the usual antimony fixation bath to develop the lake, and is then padded with a reduced vat and further treated to fix 70 the vat dye in the usual manner; for example, as above described in connection with white resists. It is much more advantageous, however, to apply the basic dyestuff in the form of the zinc lake using resorcinol as solvent, as illustrated in the following example.

75 *Example 5.*—A printing paste is made up as follows:

|                                                                                             |    |
|---------------------------------------------------------------------------------------------|----|
| 20-40 parts of Rhodamine 6G Extra (C. I. 752) or any other basic dyestuff, are dissolved in | 5  |
| 100 parts of resorcinol                                                                     |    |
| 50 parts of H <sub>2</sub> O. Then                                                          |    |
| 150 parts of 4-nitro-benzyl sodium sulfonate are added and then                             |    |
| 300 parts of gum arabic 1:1                                                                 | 10 |
| 100 parts of water                                                                          |    |
| 120 parts of tannic acid 1:1                                                                |    |
| 120 parts of zinc acetate or zinc lactate.                                                  |    |

15 After being printed with this paste, the goods are steamed, then passed directly into the reduced vat dye solution (without the antimony after-treatment), after which the goods are treated in the usual manner to fix the vat dye.

The vat dye does not "take" on the printed 20 portion of the goods, which has become dyed by the basic dye and contains the nitro-aralkyl side-chain sulfonate. The result is a printed design in the color of the basic dye on a vat dyed ground.

25 *Example 6.*—A very brilliant azo red resist may be obtained on cotton, for example, by the following procedure.

Cotton piece goods are impregnated (padded) with naphthol AS in the usual manner and then printed with a resist paste of the following composition:

|                                                                                                  | Parts  |
|--------------------------------------------------------------------------------------------------|--------|
| The diazonium compound obtained by diazotizing 18 parts of m-chlor-toluidine in the usual manner | 120 35 |
| Gum senegal                                                                                      | 300    |
| 4-nitro-benzyl sodium sulfonate                                                                  | 150    |
| Kaolin                                                                                           | 50     |
| Water                                                                                            | 300    |
| Zinc acetate                                                                                     | 80 40  |
|                                                                                                  | 1000   |

30 The nitro-aralkyl sulfonate does not interfere with the coupling of the naphthol AS and the diazonium compound, which results in a red dyeing 45 on the goods in the printed portion. After printing, the goods are well dried, steamed for four minutes, then subsequently padded by passage through an alkaline hydrosulfite solution of a reduced vat dye (e. g., one of those above mentioned), washed, soaped, rinsed and dried. The nitro-aralkyl side-chain sulfonate present in the printed portion of the goods completely resists the vat dye, thus producing a red design where 50 the goods were printed with the resist paste on a vat dyed ground where the goods were not printed.

55 Similar methods are applicable for the production of white or colored resists under sulfur 60 dyes.

65 *Example 7.*—An excellent white resist is obtained by printing the following paste:

|                                 | Parts   |
|---------------------------------|---------|
| Gum thickener                   | 300 65  |
| Manganese chloride              | 450     |
| 4-nitro-benzyl sodium sulfonate | 50      |
| Aluminum hydrate (jelly)        | 200     |
|                                 | 1000 70 |

70 After printing, the material is well dried and then dyed in a sulfur dye bath. These methods of application are well known to the art and do not need to be described in detail.

75 Excellent resist effects similar to those de-

- scribed above also may be obtained by top-printing or "blotching" the resist printed material with a vat dye printing paste, producing a so-called "resist-blotch effect". The vat dye printing paste does not "take" on the resist printed part of the goods, thus giving a design partly in the color of the resist print and partly in the color of the vat dye print.

10 *Discharge printing*

10 The use of the nitro-aralkyl side-chain sulfonates makes it possible to obtain perfect discharge effects on grounds dyed with insoluble azo dyestuffs, such as para-red or chrysoidine bister.

15 In this case the dyed fabric is simply padded in an aqueous solution composed of from 2.5 to 7 parts per 1000 of 4-nitro-benzyl sodium sulfonate or any of the other nitroaralkyl sulfonate bodies of this invention.

15 It has also been found that when used under a discharge agent the nitro-aralkyl side-chain sulfonates produce several advantageous effects. They prevent haloing, scratching and facing by oxidizing any excess discharge agent outside of the design. In addition, due to their slightly acid character, the nitro-aralkyl sulfonates act as a catalyst for certain discharges such as sodium formaldehyde-sulfoxylate which are definitely promoted by a slightly acid medium.

30 *Example 8.*—Cotton or rayon fabrics dyed with 4 per cent of Erie Black GXOO (C. I. 581) are padded through a 0.1 per cent to 1 per cent solution of 4-nitro-benzyl sodium sulfonate and dried. The fabric is then printed with a discharge printing paste containing sodium formaldehyde sulfoxylate. It is found that haloing, scratching and facing have been effectively prevented and an excellent discharge effect has been produced.

35 As above indicated, the invention is not limited to the specific examples. Thus, the procedures, ingredients and proportions thereof employed in the above specific examples may be varied. The 4-nitro-benzyl sodium sulfonate employed in the examples may be replaced by any of the other nitro-aralkyl side-chain sulfonates herein disclosed, and especially by the mono- and di-nitro-benzyl alkali metal sulfonates.

45 I claim:

- 50 1. The method of inhibiting reduction of reducible dyes on textile material which comprises treating a textile material having a reducible dye applied thereto with a nitro-aralkyl side-chain sulfonate.
- 55 2. In the process of resist coloring, the step which comprises applying to the fiber a resist composition containing a nitro-aralkyl side-chain sulfonate.
- 60 3. In the process of discharge printing, the improvement which comprises pretreating the goods with a nitro-aralkyl side-chain sulfonate.

4. In resist coloring of textile material, the improvement which comprises applying a nitro-benzyl sulfonate to the part of the material which is to resist coloring.

5. In resist coloring under vat dyes, the improvement which comprises printing the part of the material which is to resist coloring with a paste containing 4-nitro-benzyl sodium sulfonate.

6. In discharge printing, the improvement which comprises pretreating the goods with a nitro-benzyl sulfonate.

7. In discharge coloring with the aid of sodium formaldehyde sulfoxylate as a discharge agent, the improvement which comprises carrying out the discharge in the presence of an alkali-metal nitro-benzyl sulfonate.

8. In discharge printing, the improvement which comprises pretreating the material with an aqueous solution containing 4-nitro-benzyl sodium sulfonate.

20 9. In the processing of textile materials having a reducible coloring agent applied thereto by a treatment involving reducing conditions, the improvement which comprises carrying out the treatment in the presence of a nitro-aralkyl side-chain sulfonate as a reduction inhibitor.

25 10. In the processing of textile fibrous material in connection with the coloring thereof by a treatment involving subjecting a reducible coloring agent to reducing conditions in the presence of the fiber, the improvement which comprises subjecting the coloring agent and the fiber to the reducing conditions in the presence of a nitro-aralkyl side-chain sulfonate as a reduction inhibitor.

30 11. In the processing of textile fibrous material in connection with the coloring thereof by a treatment involving subjecting a reducible coloring agent to reducing conditions in the presence of the fiber, the improvement which comprises subjecting the coloring agent and the fiber to the reducing conditions in the presence of an alkali metal salt of nitro-benzyl sulfonic acid as a reduction inhibitor.

35 12. The method of inhibiting reduction of reducible dyes on textile material which comprises treating a textile material having a reducible dye applied thereto with a nitro-aralkyl side-chain sulfonate of the benzene series.

40 13. In resist coloring, the improvement which comprises printing the part of the material which is to resist coloring with a paste containing a nitro-aralkyl side-chain sulfonate of the benzene series.

45 14. In discharge coloring with the aid of sodium formaldehyde sulfoxylate as a discharge agent, the improvement which comprises carrying out the discharge in the presence of a nitro-aralkyl side-chain sulfonate of the benzene series.

50 JEAN G. KERN.

60